

1,020,345.

A. S. DWIGHT & R. L. LLOYD.

METALLIFEROUS ORE PRODUCT.

APPLICATION FILED APR. 9, 1908. RENEWED DEC. 8, 1910.

Patented Mar. 12, 1912.

2 SHEETS—SHEET 1.



Witnesses

W. F. Braun

George E. Edlin.

By

Inventor  
Arthur S. Dwight  
Richard L. Lloyd

H. H. Bliss  
Attorney

A. S. DWIGHT & R. L. LLOYD.  
METALLIFEROUS ORE PRODUCT.

APPLICATION FILED APR. 9, 1908. RENEWED DEC. 8, 1910.

1,020,345.

Patented Mar. 12, 1912.

2 SHEETS—SHEET 2.



Witnesses

W. B. Braun

George E. Edlin.

Inventors  
Arthur S. Dwight  
and  
Richard L. Lloyd  
By H. H. Bliss  
Attorney

# UNITED STATES PATENT OFFICE.

ARTHUR S. DWIGHT AND RICHARD L. LLOYD, OF NEW YORK, N. Y., ASSIGNEES, BY  
MESNE ASSIGNMENTS, TO DWIGHT & LLOYD METALLURGICAL COMPANY, OF  
JERSEY CITY, NEW JERSEY, A CORPORATION OF NEW JERSEY.

## METALLIFEROUS ORE PRODUCT.

1,020,345.

Specification of Letters Patent. Patented Mar. 12, 1912.

Application filed April 9, 1908, Serial No. 426,101. Renewed December 8, 1910. Serial No. 596,375.

To all whom it may concern:

Be it known that we, ARTHUR S. DWIGHT and RICHARD L. LLOYD, citizens of the United States, residing at New York, in the county 5 of New York and State of New York, have invented certain new and useful Improvements in Improved Metalliferous Ore Products, of which the following is a specification, reference being had therein to the accompanying drawing.

This invention relates to an improved metalliferous product adapted to be used in a blast furnace or other kind of metallurgical furnace in deriving metal therefrom, obtained by sintering the material being treated to produce the product, as for instance a finely divided ore or metalliferous material containing a combustible constituent; and the fines of sulfid ores, such as galena, pyrites, and analogous materials may be regarded as types of material from which, being properly treated, the product constituting the subject of this case may be made.

The products obtained by following the various earlier desulfurizing and sintering processes are fully understood by metallurgists skilled in the art, and it is unnecessary to here describe, in detail, either these, or the modes of treating the ores by which such earlier products are obtained. Referring especially to materials initially containing sulfur it is sufficient for present purposes, to note that the desulfurized products known in the earlier art may be regarded as of one or the other of two sorts, mechanically considered, those of one sort being masses which, throughout, are in a finely divided condition (although desulfurized), and the products of the other sort being masses each 40 consisting partly of non-uniformly sintered blocks or cakes and partly of desulfurized fines. Those products which are above referred to as masses composed of desulfurized fines are commonly obtained by using a long 45 roasting hearth or rabbling furnace wherein it is impossible to produce sintered blocks or cakes of the relatively large sizes that are necessary for good work in the blast furnace because of the fact that the agitating or rabbling treatment of the ore while on the floor or hearth of the furnace prevents the formation of such blocks or cakes. In such furnaces the fire or heated currents of gas are

generally above the ore mass and move across its upper surface, and consequently, it 55 is requisite that the mass should be frequently stirred, agitated or rabbled, so as to expose the masses or particles which are beneath the surface to the oxidizing action. The products of the other class, the second 60 above referred to, may be here typified by that obtained, during late years, from what is known in the art as the Huntington-Heberlein process. In following this mode of treatment a mass of fines, such as copper sulfid, is placed in a large vessel or receptacle, generally bowl-shaped and of such dimensions that it can hold a mass of ore fines several feet deep and several feet in horizontal diameter. The product of this process in each instance is a mass of desulfurized ore comprising two sub-masses, one of which is a large block or cake, gradually increasing in hardness from the top to the bottom, and the other sub-mass being a body of loose 70 pulverulent fines which although desulfurized are not sintered, and frequently constituting as much as a third of the entire mass, of the product. The igniting is effected by building a fire on a grate-like structure at 75 the bottom, and blowing air upward through the mass. Internal combustion is produced and travels upward through the ore from the bottom to the top. The different strata, considered horizontally, are subjected to 80 differing pressures varying with the distance from the top. The lowermost strata are subjected to the greatest pressure and have their particles pressed together more 85 tightly. As the mass is several feet (frequently three to five) in depth, the weight of the metallic ore which rests on the bottom portion of the mass is considerable. But the weights upon, and the corresponding pressures exerted by, the strata, gradually decrease upward. The air as it rises through 90 the mass becomes more and more efficient as an agitating, disturbing, or lifting agent. The weights and pressure above referred to serve to prevent the air, as it moves through 95 the lower part of the mass, from agitating or disturbing the particles in that part, and they are not prevented by it from sintering with each other. But, through the upper section (approximately the upper third of 100 the mass) the air can move with such force 105

as to agitate the particles, even forming "blow-holes" or "craters", and with the result that the ore particles in this uppermost region can not sinter, a state of substantial quiescence and rest being necessary to effect the sintering. Consequently the sub-mass at the top of the charge, considered as an entirety, in the desulfurizing receptacle, is a body of pulverulent particles which, although desulfurized, are still finely reduced and not in condition to be introduced into a blast furnace to advantage. The other sub-mass of the charge, the large sintered block at the bottom, must, after the desulfurizing stage, be broken up into small pieces or lumps preparatory to charging into the blast furnace. For this breaking much labor is required not only because of the large size of the sinter, but also because of the excessive hardness of its lower strata. The upper strata are more easily broken, and the porosity in that region is generally that which is desirable for the actions which are desired in the furnace; whereas the lower strata are much harder and more refractory, presenting greater difficulty in the breaking up, and the blocks or pieces obtained therefrom by such breaking are much less permeable to the reducing gases in a blast furnace.

In contrast with the earlier products (characterized by the above disadvantages) derived from following the commonly used processes of desulfurization and sintering, we have succeeded in furnishing for the blast furnace a desintered product of such nature that it is, throughout, uniformly the same in porosity, permeability, and hardness, along horizontal lines and along vertical lines, and can be produced in indefinitely large quantities, which are, throughout, uniform in the above respects.

While we have referred especially to materials initially containing sulfur and requiring desulfurization, it will nevertheless be understood that our invention is not thus limited and that our improved product may be formed of any metal bearing or other material capable of being sintered.

We effect the sintering of the ore while it is arranged in relatively thin, uniformly distributed, masses or layers. And the important results are that there occurs complete sintering of the entire mass of fines in the stratum or layer, air being conducted through it in such way that none of its particles are agitated or disturbed to an extent to prevent complete and uniform sintering. The internal combustion resulting from the oxidizing of the sulfur or other combustible constituent insures a uniform sintering action from one surface of the mass to the other. By suitably holding the ore, and causing the air to travel through it in a suitable way, the retaining of the

particles in the quiescent state can be secured even though the layer is thin and does not have any part of its mass exert any considerable weight upon another part; the sintering, here, not depending upon the action of gravity or upon the pressure of the upper part of the ore mass upon the lower part.

While the characteristics incident to our product are not necessarily limited to a sinter of any precise dimensions or composition, we have found that the material for the blast furnace is in the best condition when produced from a layer or stratum of fines which is from two to five inches in thickness. We prefer to manufacture this product in an apparatus which carries the stream or stratum of ore, more or less nearly continuously, from point to point, while the sintering action is occurring; and because of treating it while it is thus in motion, there is economy in time and labor which more than compensates for what would apparently be a loss due to the thinness of the mass. To obtain our product in this way, use can be made of any of several forms of mechanism. In order that the present invention may be fully understood we have selected for illustration in the drawings herein one of the simpler forms of mechanism for this purpose, although it is to be understood that neither the mechanism nor the method of using it enters essentially into the present subject matter.

Figure 1 is a side view, partly in section, of an apparatus in which our improved metal bearing products can be made. Fig. 2 is a plan view. Fig. 3 is a perspective view of a sample of the product, the right hand end illustrating the appearance of the interior when the sample is cut on a transverse plane.

Inasmuch as an apparatus of the kind generally indicated more or less conventionally in the drawings is described in our Patent No. 916,394 issued March 23, 1909, it is not necessary to describe it here in all of its details. Suffice it to say that T indicates an ore-carrying and supporting element which is drum-like in construction, having flange walls *t*, with inward projecting ring-sections *t*<sup>1</sup> and the ore-supporting part N, the latter being formed of perforated or barred sections clamped in place. The drum is supported by means of rings O which rest upon and are actuated by rollers P and Q.

F indicates the hopper for the ore, the latter passing if desired in a continuous stream to the space between the side flanges *t* and above the perforated support N. The ore is preferably smoothed at its top surface and the layer is preferably from two to six inches in depth, this being in contradistinction from the deep bodies (generally from

four to five feet in depth) of fines placed in the pots or receptacles when the earlier processes above referred to are followed.

H is a wind-box or air-trunk in the chamber or space in the interior of the drum. It communicates with an exhaust mechanism through a pipe h.

K is a chute for separating and withdrawing the sintered ore from the drum.

10 To form our improved product with this apparatus the ore which is stored in the hopper is delivered, as above set forth, to the drum, and the latter is slowly revolved.

15 At G the sulfur ingredients or other combustible elements of the mass are ignited, there being at this transverse line a gas pipe from which the gas jets issue toward the top surface of the ore. The air suction apparatus being set in operation, air is drawn 20 downward through the burning layer and the gases are taken into the box H and withdrawn thence by the exhaust mechanism. Inasmuch as the air moves downward through the ore, it has no lifting or disturbing action upon it. The particles at 25 the upper surface of the stream remain in quiescence relatively to each other, and those at the lower surface are held against displacement by the holder (the perforated 30 floor, the grate sections, or the like) and sintering is not interfered with. By the time the ore reaches the limit of the air box the sintering is completed and the sinter 35 is ready for removal. As the relatively thin solid mass reaches the take-off device at K, it is separated from the drum and slides down the chute, the action at this point in the apparatus automatically breaking the sinter mass into relatively small 40 blocks or cakes which can be readily picked up by the operatives or loaded upon vehicles and transported to the blast furnace ready for charging therein. As the quiescence of the particles extends from the top to the 45 bottom of the mass the sintering is uniform through the entire layer, and as there is no considerable pressure experienced by one stratum of the ore from the weight of the superincumbent strata there results a practically uniformity in the porosity of the sinter not only along lines longitudinal of its mass but on transverse lines and on vertical lines. The lower stratum is no harder 50 or more indurated than are the strata above it, for the stream being only a few inches in thickness there is no pressure-generating weight upon the lower particles. By reference to Fig. 3 some of the physical characteristics of this desulfurized sinter will be 55 found conventionally delineated. As the layer of material being sintered is initially made practically smooth, that is, for instance, as smooth as results from feeding the material to a moving support 60 to form a layer of uniform thickness, and

as the layer rests upon a smooth though perforated or apertured support, the resulting sinter has a top surface and a bottom surface which are also correspondingly smooth and well defined, there being in 70 these surfaces uniformly distributed and uniformly sized pores or gas passages. And as the layer is comparatively thin, the texture and consistency of the sinter in respect to its porosity and permeability are 75 uniform from the top surface, through the body, to the bottom surface. This sintered product is not only of substantially uniform porosity but is self-sustaining and capable of maintaining its shape though subject to 80 considerable weight or pressure, which insures that when introduced into a smelting furnace the oxidizing, reducing, or other gases which are forced through the furnace and the material contained therein readily 85 pass through the body of each piece of the sintered product as well as through masses thereof which may be comprised in the layers or strata of the furnace charge, thus bringing the heat and the reducing or oxidizing gases into very close and intimate 90 relation with the metal being treated and contained in the sintered masses. The blocks or pieces of sintered material produced according to our process herein 95 described are, owing to their porosity, relatively light and of relatively low specific gravity as compared with its own metallic and other constituents.

While we have referred to our improved 100 product as normally having its oppositely disposed surfaces relatively smooth and well defined, it will be understood that many of the advantageous features incident to our invention are present in those 105 smaller fragments of material which may result from the breaking up of initially complete and regularly formed cakes. In fact, in many cases the smaller bodies are found preferable for treatment in a smelting furnace. The partial breaking up or disintegration of the cakes in those cases where it is found to be desirable or unavoidable, is not to be construed as removing the product from within the scope of our invention. On the contrary, our invention is to be understood as relating broadly to uniformly porous sinter cakes or blocks initially having relatively smooth and well defined surfaces, and this irrespective of the 110 treatment which the cakes may undergo subsequent to formation and after leaving the perforated grate sections upon which they are first supported.

What we claim is:

1. The herein described metalliferous product adapted for use in obtaining metals in a smelting furnace, the same being a block of sintered ore having normally smooth top and bottom surfaces and uni- 130

formly porous between the said surfaces, substantially as set forth.

2. The herein described metalliferous product adapted for use in obtaining metals in a smelting furnace, it consisting of a relatively thin block or cake of ore having its particles sintered together from the top surface to the bottom surface and being uniformly porous and permeable to gases at the said surfaces, and throughout the body between them, substantially as set forth.

3. The herein described metalliferous product adapted for use in obtaining metal

in a smelting furnace or equivalent, it being a relatively thin block or cake of desulfurized, sintered ore with relatively smooth upper and lower surfaces, and a body part between them, said surfaces and body being uniformly porous and permeable to gases, substantially as set forth.

In testimony whereof we affix our signatures in presence of two witnesses.

ARTHUR S. DWIGHT.  
RICHARD L. LLOYD.

Witnesses:

H. J. STEBLI,  
GRACE ELIZABETH SEYMOUR.

Correction in Letters Patent No. 1,020,345.

It is hereby certified that in Letters Patent No. 1,020,345, granted March 12, 1912, upon the application of Arthur S. Dwight and Richard L. Lloyd, of New York, N. Y., for an improvement in "Metalliferous Ore Products," an error appears in the printed specification requiring correction as follows: Page 2, line 36, for the word "desintered" read *sintered*; and that the said Letters Patent should be read with this correction therein that the same may conform to the record of the case in the Patent Office.

Signed and sealed this 16th day of April, A. D., 1912.

[SEAL.]

C. C. BILLINGS,

Acting Commissioner of Patents.

formly porous between the said surfaces, substantially as set forth.

2. The herein described metalliferous product adapted for use in obtaining metals in a smelting furnace, it consisting of a relatively thin block or cake of ore having its particles sintered together from the top surface to the bottom surface and being uniformly porous and permeable to gases at the said surfaces, and throughout the body between them, substantially as set forth.

3. The herein described metalliferous product adapted for use in obtaining metal

in a smelting furnace or equivalent, it being a relatively thin block or cake of desulfurized, sintered ore with relatively smooth upper and lower surfaces, and a body part between them, said surfaces and body being uniformly porous and permeable to gases, substantially as set forth.

In testimony whereof we affix our signatures in presence of two witnesses.

ARTHUR S. DWIGHT.  
RICHARD L. LLOYD.

Witnesses:

H. J. STEBLI,  
GRACE ELIZABETH SEYMOUR.

Correction in Letters Patent No. 1,020,345.

It is hereby certified that in Letters Patent No. 1,020,345, granted March 12, 1912, upon the application of Arthur S. Dwight and Richard L. Lloyd, of New York, N. Y., for an improvement in "Metalliferous Ore Products," an error appears in the printed specification requiring correction as follows: Page 2, line 36, for the word "desintered" read *sintered*; and that the said Letters Patent should be read with this correction therein that the same may conform to the record of the case in the Patent Office.

Signed and sealed this 16th day of April, A. D., 1912.

[SEAL.]

C. C. BILLINGS,

Acting Commissioner of Patents.

It is hereby certified that in Letters Patent No. 1,020,345, granted March 12, 1912, upon the application of Arthur S. Dwight and Richard L. Lloyd, of New York, N. Y., for an improvement in "Metalliferous Ore Products," an error appears in the printed specification requiring correction as follows: Page 2, line 36, for the word "desintered" read *sintered*; and that the said Letters Patent should be read with this correction therein that the same may conform to the record of the case in the Patent Office.

Signed and sealed this 16th day of April, A. D., 1912.

[SEAL.]

C. C. BILLINGS,

*Acting Commissioner of Patents.*